

March 13, 1928.

1,662,506

G. H. MANSFIELD

METHOD OF ROLLING STAYBOLT IRON

Filed Nov. 25, 1925

Fig. 1



Fig. 2



Fig. 3



Fig. 4



Fig. 5



Fig. 6



WITNESSES

Geo. F. Burnett  
L. Schumacher

INVENTOR

George H. Mansfield

Patented Mar. 13, 1928.

1,662,506

# UNITED STATES PATENT OFFICE.

GEORGE HENRY MANSFIELD, OF CUYAHOGA FALLS, OHIO.

## METHOD OF ROLLING STAYBOLT IRON.

Application filed November 25, 1925. Serial No. 71,364.

This invention relates to new principles introduced to the rolling, hammering, pressing, or otherwise shaping of hollow-staybolt iron or steel bars and has for one of its objects the working or rolling of a hollow bar from an original hollow pile; another object being to produce such a bar substantially seamless, still another to materially increase the tonnage production from a given amount 10 of fuel and labor and hence reduce the cost per pound.

Referring to the accompanying drawings, in which similar parts are similarly designated, I show in Figure 1 a cross-sectional view of a hollow pile of sectional iron bars arranged substantially in the formation of a tube; in Figure 2 a steel mandrel designed to be used by insertion into the hollow pile to control the size and contour of the hole 20 thereof; in Figure 3 an illustration of the manner in which the hollow pile is entered into the rolls of a rolling mill and of the manner of inserting the said mandrel; in Figure 4 a longitudinal cross-section of an 25 iron container or tube containing a refractory core; Figure 5 a hollow billet evolved from the said hollow pile, having the core of Figure 4 inserted therein; and in Figure 6 a finished hollow staybolt bar.

Proceeding to explain the invention in more exact detail, in the construction of the hollow pile of Figure 1 I employ, preferably, four sectional bars curved in such a manner that two of them butted against each other 35 form a tubular shape and constitute the inner layer 2 of the hollow pile; after which a second or outer layer 1 is provided by enveloping the said inner layer 2 with similarly curved sectional bars. The hollow pile thus 40 formed is charged into a heating furnace and brought to a welding heat, when it is removed from the furnace and rolled through reducing rolls of a rolling-mill. Such rolls are illustrated in cross-sectional views 13 of 45 Fig. 3, with collars 14. The operation is effected by setting the heated hollow-pile upon a suitable bed as indicated by dotted outline 14, at which juncture an operative inserts mandrel 4 into hole 3 to an extent that 50 mandrel-tip 5 reaches a location within the pile exactly at a line centrally between the axes of rolls 13, whereupon another operative enters the pile into the said rolls 13, resulting in reduction of its cross-sectional diameter 55 as indicated at 20, while the hole 3 is correspondingly reduced 8 to the diameter of

mandrel-tip 5. By provision of a fixed stop upon mandrel-bed 18 and a shoulder-plate 6 on mandrel 4, the latter is prevented from accompanying the pile through the rolls, the 60 rolls, in effect, drawing the pile off the mandrel. Handle 7 is provided on the mandrel 4 for grasping by the operative. In Figure 3 is shown a partially cut-out section to clearly illustrate the longitudinal cross-section 65 of said pile and the generous clearance space 3 between the mandrel 4 and inner layer 2 of pile, and which facilitates the entry of the mandrel 4. I may give the pile additional passages through the rolls over mandrels, 70 each successively smaller in diameter. The number of such operations is governed by the outside and inside diameters which are desired in the finished bar. After the passages over mandrels, when the pile is thoroughly welded into an integral mass of iron, it has become an evolved hollow billet as shown at 15 of Fig. 5, into the hollow of which is inserted a core-bar of which a longitudinal cross-section is shown in Fig. 4, 80 consisting of a tubular container 9 holding a refractory 10, plugged 11 at the ends with edges of container 9 bent over as at 12 to hold securely the plugs 11. Again in Fig. 5 I show a partially cut-out section of billet 15 85 to illustrate the disposition of core-bar 9 within said billet 15, which thereupon is rapidly rolled down through the successive passes of ordinary rolling-mill rolls to the desired diameter of the finished bar 16 of Fig. 6. 90 In these reducing operations the core 10 is reduced in cross-section in proportion to the wall of the billet, evolving into a finished bar of relatively thick wall and small core 95 17, which latter may be extracted in any desired manner, such as drilling, reaming, or water or air pressure.

It is obvious that substitutes for the hollow pile may be used, such as drilled, pierced or forged masses of iron, and yet remain 100 within the scope of my invention embodying the combination of the principles of the mandrels and the core.

It is further obvious that the core is not restricted to the combination of a core with 105 in a container, as any core substance possessing an adequate heat-resisting property and reasonably rigid form for convenient insertion into the hole of the pile or billet, would equally carry out the spirit of my 110 invention. Nor must it be necessarily a refractory, since if a cold container be used,

and kept out of the furnace until the pile is drawn therefrom, it would be practicable to employ copper or any other metal or substance of fairly high heat-resisting property within the core container; or again, such copper bar may be used unencased, by squirting a stream of cold water through the hole of the pile or billet to chill or materially reduce the temperature of the immediate inner wall to such an extent as will not melt the copper, which, retaining its solidity, would occupy its proportion of the cross-sectional area in the successive operations of reduction. In the event of using such metallic core, I would preferably extract it from the finished bar by heat, as in an electric furnace, to a degree that the copper would melt and flow out, without, however, reaching the critical point of heat of the iron itself.

It is further obvious that various core refractories can be used, such as silica sand, mica, fireclay, carbon, and the various products of electric or other high-temperature furnaces, such as "carborundum," "aloxite," "siloxicon," calcined magnesite, et al.

My invention embraces the principle of exposing the unincumbered pile to the furnace heat, without core or anything whatever inside; thereby the entire inner surface, along with the outer surface, is exposed directly to the heat, which in effect saves practically 50% of the fuel required to heat a given tonnage of iron, hence achieving a wholly new condition of economy.

It is obvious that various substitute core materials might be used by this method, such

as hardwood, sawdust, etc., since, while such materials are combustible, yet the core-container 9 is kept from the heated iron until inserted into billet 15, thereby acting as a shield against heat reactions of the core.

It is also obvious that ice might be employed as a core, since the sole object of the core is but to momentarily preserve a relative rigidity and resistance of core-container 9 to the compressive action of the roll passes.

Having thus described my invention what I claim as new and desire to secure by Letters Patent is:

1. The method of making hollow stay-bolts which consists in assembling metal pieces to form a hollow pile, heating said pile, welding said pieces together and reducing the cross sectional diameter of said pile in successive stages, controlling the diameter of hole in the pile with mandrels during the first stages of reduction and controlling the diameter of hole by a core in the last stages of said reduction, said core being inserted in said pile while said pile is still hot.

2. The method of making hollow stay-bolts which consists in assembling metal pieces to form a hollow pile, heating said pile, welding said pieces together and reducing the cross sectional diameter of said pile in successive stages, controlling the inner diameter of said pile in the first stages of reduction with mandrels and controlling the inner diameter in the last stages of reduction by a core, said core being inserted in said pile after said pile has been heated.

GEORGE HENRY MANSFIELD.